

## UNITED STATES PATENT OFFICE

2,251,774

## LUBRICANT ADDITIVE

Meyer S. Agruss and George W. Ayers, Jr., Chicago, and Hans Schindler, Evanston, Ill., assignors to The Pure Oil Company, Chicago, Ill., a corporation of Ohio

No Drawing. Application December 28, 1939,  
Serial No. 311,244

26 Claims. (Cl. 252—59)

This invention relates to lubricating oils and to processes for improving their properties and more particularly to the production of lubricating oils having reduced pour tests.

Lubricating oil stocks, particularly those derived from paraffinic and mixed base crudes, contain appreciable amounts of wax and, therefore, have a relatively high pour test unless a substantial amount of this wax is removed. The wax may be removed by various methods such as cold settling, filtration or centrifuging. However, such processes are expensive and even after such processes have been practiced, lubricating stocks may still retain appreciable amounts of wax and may have pour tests above 15° F. and even up to about 50° F. The removal of additional quantities of wax from these stocks necessitates further expensive processing. Furthermore, complete removal of wax from an oil frequently causes the removal of other materials valuable as lubricants, as well as causing an undesirable increase in the rate of change of the viscosity of the oil with temperature, that is, such removal of wax results in a lower viscosity index of the oil. It is therefore of advantage to add to the oil a material which will reduce the pour test without it being necessary to remove all or substantially all of the wax. Materials such as wax, which are generally presumed to cause high pour point tests in lubricating oil, apparently act by partly crystallizing from the remainder of the oil in such a way that a lattice or honeycomb interlacing or interlocking structure is formed which prevents the free flow of the oil.

One method of lowering the pour point of oil depends not on removing the materials responsible for such lattice structure, but on adding to the oil containing all or only part of them, such a material as will completely or partially inhibit or interfere with the formation of such a structure and thus permit the oil to flow freely at lower temperatures than it would without the added material.

Although it is believed that the foregoing discussion is a reasonably accurate explanation of the function of pour depressants, it is not desired that this invention be limited by this theory of how the materials covered in this invention act to lower the pour point. The use of addition agents within the scope of this invention is contemplated particularly for lowering the cold test of partially dewaxed oils, though the additive materials herein described are suitable for use with any hydrocarbon oil whether wholly de-

waxed or whether containing all of its natural wax content. For example, a substantial lowering of the cold test of the oil may be obtained relatively economically by pressing the wax bearing oil at a relatively high temperature, such as for example, approximately 60° F. whereby a portion of the wax is removed and then adding material prepared in accordance with this invention to reduce the pour test of the pressed oil.

- 10 The refrigeration required to obtain this temperature in commercial practice is not particularly great. A large lowering of the cold test of the oil may be obtained in this way at little expense in contrast to the considerably increased cost of lowering the cold test by operating the pressing process at a sufficiently low temperature to obtain the same pour test. It is obvious that greater quantities of the addition agents will be required to lower the pour point of a wholly undewaxed oil than for one which has been partially dewaxed. Thus in the preferred embodiment of the invention it is preferred to partially dewax the oil by pressing at relatively high temperature or centrifuging or some other conventional method, since the cost of the high temperature dewaxing operation plus relatively large quantities of pour depressant is usually much less than the cost of low temperature dewaxing operations plus relatively small quantities of pour depressant. Rather than process at low temperature, it is preferred to add one or more of the addition agents herein described so as to obtain the same lowering of the pour point by this less expensive method and without loss of yield of lubricating constituents.

35 An object of the present invention is to provide lubricating oils of low pour test.

Another object is to provide new pour point depressing materials to be added to lubricating oils.

40 Other objects and advantages will appear from the detailed description which follows.

This invention contemplates the addition to mineral oils of products resulting from the condensation of petroleum resin with halogenated, preferably chlorinated hydrocarbons, particularly those hydrocarbons of the paraffin series. Condensation may be effected by any of the well known condensing agents such as metallic halides, especially aluminum chloride. A convenient and economical source of such paraffin hydrocarbons may be petroleum wax such as the usual paraffin wax or petrolatum which is obtained in the course of conventional refining methods applied to the manufacture of lubricating oils.

Resins suitable for the condensation reaction are those resins obtained from spent or partially spent adsorbents which have been used in decolorizing operations on petroleum oils such as neutral oils, bright stocks and cylinder stocks. Such resins may be conveniently obtained by extracting the spent adsorbents with chloroform or a mixture of benzol and alcohol or a similar solvent. In order to reduce the amount of oil in the resins, the spent adsorbent is preferably washed with petroleum naphtha prior to the extraction with benzol and alcohol or chloroform. The resin may be readily separated from the solvent-resin solution by distillation and is obtained as a dark brown viscous fluid. If the petroleum oil which is decolorized by contact with the adsorbent contains excessive asphaltic material, it may be desirable to separate at least a portion of this asphaltic material prior to contact with the decolorizing adsorbent. This may be readily accomplished by any of several well-known de-asphaltizing methods, for example, by the use of propane.

Pour point depressors in accordance with this invention have been prepared by chlorinating petrolatum of, for example, about 140° F. melting point, with chlorine gas until the petrolatum contained approximately 10% to 25% chlorine by weight. The temperature was controlled during the chlorination operation so that the temperature was not substantially in excess of 300° F. The chlorinated product was mixed with hydrocarbon resin obtained from partially spent decolorizing clay which had been used to decolorize Pennsylvania cylinder stock. This resin was obtained by first washing the spent clay with naphtha to remove any oil that may have been present and then extracting the naphtha-washed clay with chloroform. The chloroform was distilled from the resin-chloroform solution and the resin obtained as a dark brown, sticky fluid of approximately 1.02 specific gravity and about 590 seconds Saybolt Universal viscosity at 210° F. The chemical condensation of the chlorinated petrolatum and resin was effected by adding anhydrous aluminum chloride to the mixture as a condensation catalyst and gradually heating to a temperature of approximately 200° F. to 220° F. This temperature was maintained until the reaction was complete, which in this case was about forty-five minutes. The completeness of the reaction may be readily determined by the cessation of the evolution of hydrogen chloride gas. The temperature at which the condensation reaction may be carried out may vary considerably, but preferably should not exceed 300° F. The amount of aluminum chloride used was 10% by weight based on the resin. The amount of aluminum chloride used may vary between wide limits, but in general it is preferred to use approximately 2% to 10% by weight of aluminum chloride based on the resin. The condensation reaction was carried out under conditions of constant agitation in carbon tetrachloride which functioned solely as a solvent to diminish the viscosity of the mixture. When the reaction was complete, insoluble reaction products were removed by water washing. The reaction product was readily separated from the carbon tetrachloride by fractional distillation. The proportion of hydrocarbon resin to chlorinated petrolatum which may be used may be varied between rather wide limits. In general it has been found that most satisfactory results were obtained by using

approximately three parts of hydrocarbon resin to two parts of chlorinated petrolatum.

The effect of the addition of an additive in accordance with this invention and prepared as set forth in the preceding paragraph, on the pour point of a high-grade lubricating oil consisting of a blend of bright stock and neutral oil may be readily seen by reference to Table I:

Table I

|                           | A. S. T. M. pour test, °F. |
|---------------------------|----------------------------|
| Mineral oil, S. A. E. 20  | +25                        |
| Mineral oil + 1% additive | - 5                        |

10 15 The additive shown in Table I was prepared by condensing three parts of resin with two parts of petrolatum which contained approximately 10% chlorine.

20 25 From the above table the efficiency of additive prepared in accordance with this invention is fully demonstrated. While in the foregoing tests 1% of the additive was blended with the lubricant, this amount may be varied within rather wide limits depending upon such factors as the quality and pour test of the original lubricant and composition of the additive.

30 Although the foregoing description sets forth a preferred embodiment of the invention and a preferred mode of carrying the same into effect, it will be readily apparent to those skilled in the art that many variations and modifications may be made therein without departing from the spirit of the invention.

We claim:

35 1. A lubricant comprising a major portion of hydrocarbon oil and a minor portion of hydrocarbon resin-halogenated hydrocarbon condensation product, said hydrocarbon resin having been obtained from partially spent decolorizing adsorbent.

40 45 2. A lubricant comprising a major portion of hydrocarbon oil and a minor portion of hydrocarbon resin-chlorinated hydrocarbon condensation product, said hydrocarbon resin having been obtained from partially spent decolorizing adsorbent.

50 3. Lubricant in accordance with claim 2 in which the proportion of hydrocarbon resin to chlorinated hydrocarbon is approximately 3 to 2.

55 4. A lubricant comprising a major portion of hydrocarbon oil and a minor portion of condensation product of halogenated paraffinic hydrocarbon and hydrocarbon resin obtained from partially spent decolorizing adsorbent.

55 5. A lubricant comprising a major portion of hydrocarbon oil and a minor portion of condensation product of chlorinated paraffinic hydrocarbon and hydrocarbon resin obtained from partially spent decolorizing adsorbent.

60 6. Lubricant in accordance with claim 5 in which the resin is obtained from partially spent decolorizing adsorbent which has been used for decolorizing residual petroleum oils.

65 7. Lubricant in accordance with claim 5 where the condensation product is present in the proportion of about 0.1% to 10%.

70 8. Lubricant in accordance with claim 5 where the chlorinated paraffinic hydrocarbon is chlorinated petrolatum.

75 9. A lubricant comprising a major portion of hydrocarbon oil and a minor portion of condensation product of chlorinated paraffinic hydrocarbon containing approximately 10% to 25% chlorine and hydrocarbon resin obtained from partially spent decolorizing adsorbent.

10. Lubricant in accordance with claim 9 in which the proportion of hydrocarbon resin to chlorinated paraffinic hydrocarbon is approximately 3 to 2.
11. Lubricant in accordance with claim 9 in which the chlorinated paraffinic hydrocarbon is chlorinated petrolatum.
12. Lubricant in accordance with claim 9 in which the condensation product is present in the proportion of about 0.1% to 10%.
13. A lubricant additive useful in reducing the pour test of relatively high pour test lubricating oils comprising the condensation product of halogenated paraffinic hydrocarbon and hydrocarbon resin obtained from partially spent decolorizing adsorbent.
14. Product in accordance with claim 13 where the paraffinic hydrocarbon is chlorinated.
15. A lubricant additive useful in reducing the pour test of relatively high pour test lubricating oils comprising the condensation product of chlorinated petrolatum and hydrocarbon resin obtained from partially spent decolorizing adsorbent.
16. Product in accordance with claim 15 where the chlorinated petrolatum contains approximately 10% to 25% chlorine.
17. Method of preparing a pour depressant comprising chemically reacting halogen with hydrocarbon, mixing the halogenated hydrocarbon with hydrocarbon resin obtained from partially spent decolorizing adsorbent and a condensation agent, heating the mixture to elevated temperature and maintaining the temperature for a sufficient time to effect condensation of the halogenated hydrocarbon and hydrocarbon resin and separating the condensation product from the reaction mixture.
18. Method in accordance with claim 17 in which the halogen is chlorine.
19. Method of preparing a pour depressant comprising chemically reacting chlorine with paraffinic hydrocarbon, mixing the chlorinated hydrocarbon with hydrocarbon resin obtained from partially spent decolorizing adsorbent which has been used to decolorize petroleum oils, and a condensation agent, heating the mixture to elevated temperature and maintaining the temperature for a sufficient period of time to effect condensation of the chlorinated hydrocarbon and hydrocarbon resin and separating the condensation product from the reaction mixture.
20. Method in accordance with claim 19 in which the mixture is heated to a temperature of approximately 200° F. for about forty-five minutes.
21. Method in accordance with claim 19 where the paraffinic hydrocarbon is petroleum wax and the proportion of hydrocarbon resin to chlorinated wax in the condensation product is approximately 3 to 2.
22. A lubricant additive useful in reducing the pour test of relatively high pour test lubricating oils comprising the condensation product of halogenated hydrocarbon and hydrocarbon resin obtained from partially spent decolorizing adsorbent.
23. A lubricant additive comprising the condensation product of chlorinated hydrocarbon and hydrocarbon resin obtained from adsorbent clay which has been used for decolorization of Pennsylvania type lubricating oil stock.
24. Additive in accordance with claim 23 where the hydrocarbon resin is obtained from the adsorbent clay by extraction with chloroform.
25. Additive in accordance with claim 23 where the hydrocarbon which is chlorinated is petroleum wax.
26. Additive in accordance with claim 23 where the hydrocarbon which is chlorinated is petroleum wax and the hydrocarbon resin is obtained from the adsorbent clay by extraction with chloroform.

MEYER S. AGRUSS.  
GEORGE W. AYERS, JR.  
HANS SCHINDLER.